

April 11, 1933.

W. F. HENDERSON

1,903,622

METHOD OF PRODUCING CELLULOSE ARTICLES

Filed Nov. 26, 1930



### Inventor.

William F. Henderson.

William Henderson  
By Wrenforth, Lee, Thornton & Wiles. Atlys.

## UNITED STATES PATENT OFFICE

WILLIAM F. HENDERSON, OF CHICAGO, ILLINOIS, ASSIGNOR TO THE VISKING CORPORATION, OF CHICAGO, ILLINOIS, A CORPORATION OF VIRGINIA

## METHOD OF PRODUCING CELLULOSE ARTICLES

Application filed November 28, 1930. Serial No. 498,487.

The invention relates to apparatus for producing articles from cellulose, and more particularly to apparatus for producing cellulose tubes or sausage casings.

- 5 In the preferred embodiment of the invention, the cellulose tubing is preferably formed from viscose which is obtained by practicing the method briefly described in U. S. Letters Patent No. 1,612,508, granted 10 December 28, 1926, to William F. Henderson and Harold E. Dietrich. The viscose is extruded through an annular orifice and is subjected to one or more solutions so that it again becomes cellulose or cellulose hydrate. 15 The tubing is then washed in water and subsequently treated with a hygroscopic agent, such as glycerine, to prevent it from drying to such an extent that it will crack.

The present invention relates particularly 20 to improved apparatus for and an improved method of washing the tubing after it has been immersed in the hardening solutions.

In practicing the improved method, the tubing is washed in a series of wash tanks 25 holding warm water at different temperatures, the arrangement being such that the tubing is thoroughly cleansed of the by-products resulting from the reaction of the viscose and the hardening baths or solutions. The 30 temperature of the water in the several tanks is such that the gases evolved do not accumulate more rapidly than they can diffuse through the cellulose wall and, therefore, there is no excessive overstretching of the 35 tubing and it is not deformed.

Other objects and advantages of the invention will become apparent as the following detailed description progresses, reference being had to the accompanying drawing, 40 wherein:

Figure 1 is a somewhat diagrammatic view of a section taken through apparatus which embodies the invention.

Fig. 2 is an enlarged fragmentary section 45 taken through one of a plurality of wash tanks shown in Fig. 1, and

Fig. 3 is a diagram of electrical apparatus which is utilized to control the temperature of the water in the wash tanks.

50 Referring for the present to Fig. 1 wherein

a preferred embodiment of the invention is illustrated somewhat diagrammatically, the reference character 10 designates generally apparatus for extruding viscose through an annular orifice to form cellulose tubing 55 which is shown at 11, the tubing being extruded into a coagulating or regenerating bath 13 and being advanced over a roller 14 to a tank 15 holding a coagulating or regenerating solution. From the receptacle 15 60 the tubing is advanced to a receptacle 16 which holds an aqueous solution of the coagulating or regenerating agents, these agents being carried over into the solution from the receptacle 15 by the tubing. The 65 tubing is then advanced from the receptacle 16 through a plurality of wash tanks 17, 18, 19 and 20, and thence into a receptacle 21 which holds a hygroscopic agent, preferably 70 glycerine. Idler rolls 23 in the receptacles 15, 16, 17, 18, 19, 20 and 21 and driven rolls 24 disposed above these receptacles guide and advance, respectively, the tubing through the several receptacles.

Various solutions are employed in the extruding apparatus and in the receptacle 15 for hardening the viscose. In practicing one embodiment of the invention an aqueous solution of 8 to 10% of sulfuric acid and 12 to 16% of sodium sulfate is employed in the 75 extruding apparatus, and in another embodiment of the invention an aqueous solution of 2.5% to 3.5% sulfuric acid, 14 to 17% of ammonium sulfate, and 12 to 16% of sodium sulfate is employed in the extruding 80 apparatus, the extruding apparatus being provided with a receptacle 25 which holds these solutions. In the event the second solution is employed in the receptacle 25, a regenerating solution is employed in the receptacle 15. 85

The reaction of the acidified salt baths and the viscose produces several substances, such as sodium sulfate, sodium bisulfate, hydrogen sulfide, colloidal sulfur, etc., all of 90 which must be washed out of the regenerated cellulose film before it is dried. It is for this purpose that the tubing is conveyed through the wash tanks 17, 18, 19 and 20, which tanks preferably hold running water. 100

Hot water will remove these bi-products from the film or tube much more quickly than cold water. However, if the film or tube is carried into hot water immediately after leaving the acidified regenerating bath an inferior product may result. The acid which is associated with the regenerated film soon imparts a permanent acidity to the water in the first wash tank if the water is not changed often enough to prevent such acidity. If the temperature is high, this acid exerts a weakening effect on the cellulose film. Volatile substances formed by the action of the acid on the viscose are quickly driven out of the film when it is immersed in hot water, and, under certain conditions, may cause minute gas bubbles to be formed in the film itself. These volatile substances are probably hydrogen sulfide, carbon disulfide and carbon dioxide. The production of these volatile biproducts presents the greatest difficulty when the cellulose product is in the form of a seamless tube. Here, a substantial rise in temperature following the generate or cellulose when the tube is lead into hot water causes an inflation of the tube by the gases trapped inside. Under these conditions, the gases accumulate more rapidly than they can diffuse through the cellulose wall and serious overstretching and deformation results.

Regenerated cellulose films are subject to severe shrinkage during the regenerating operation and during subsequent washing stages, and the use of hot water accelerates this shrinkage. The application of hot water immediately after the acid treatment causes such severe and sudden shrinkage that frequent breakage may occur.

The present invention permits the use of hot water for washing the regenerated cellulose films or tubes without encountering the difficulties mentioned above. Thus, the temperature of the water in the wash tanks 17, 18, 19 and 20 is gradually raised, beginning with water at about the same temperature as that maintained in the acid tank and ending in the final wash tank 20 with hot water. In a preferred embodiment of the invention, the water in tank 17 is held at approximately 20° C., the water in the second tank 18 is held at about 30° C., the water in the tank 19 is held at about 35° C., and the water in the tank 20 is held at 50° C., or even higher.

As indicated above, the water in the tanks 17, 18, 19, and 20 is preferably changed at frequent intervals or continuously, thus pipes 17a, 18a, 19a and 20a are adapted to discharge water into the receptacles 17, 18, 19 and 20, respectively, the overflow being carried off by pipes 17b, 18b, 19b and 20b, respectively. If it is so desired, each of the tanks 17, 18, 19 and 20 may be connected to a larger tank so that the water may be circulated continuously. Such construction permits the tem-

perature of the water to be readily controlled.

In the preferred embodiment of the invention, means is preferably associated with each of the tanks 17, 18, 19 and 20 to control the temperature of the water therein. In this instance, the controlling means comprises heating devices 30, 31, 32 and 33 disposed in the tanks 17, 18, 19 and 20, respectively, the heating devices being preferably electrical resistances. The resistances are connected to a suitable source (not shown) of electrical energy, as illustrated in Fig. 3. The resistances 30, 31, 32 and 33 are controlled by thermostatic devices 35, 36, 37 and 38, respectively, which are preferably identical in construction. The thermostatic device 35 is illustrated in detail in Fig. 2 and comprises, in this instance, a diaphragm 39 holding a quantity of some suitable volatile fluid which will expand when it is heated. The diaphragm is carried by a bracket 40 mounted in the tank 17, the diaphragm being positioned beneath the surface of the water in the tank.

The free end of the diaphragm 39 is connected by a post 41 to a lever 42 which is pivoted intermediate its ends to a bracket 43 carried by the tank 17. A member 44, depending from one end of the lever 42, is adapted to depress a metallic spring member 45 when the diaphragm 39 expands. The spring member 45 carries a contact point 46 engageable with a contact point 47 carried by a spring member 48. The spring members 45 and 48 are insulated from each other and are mounted in a housing 49 secured to a wall of the tank 17. A set screw 50 screw-threaded through one of the walls of the housing 49 engages the spring member 48 and is adapted to bring it into a plurality of adjusted positions. Thus, the spring member 48 tends to flex in an upward direction and the screw 50 may be manipulated against this action to bring the contact point 47 into any desired position with respect to the contact point 46. The spring member 45 also tends to spring upward so as to bring the contact point 46 into engagement with the contact point 47. Obviously, the apparatus may be adjusted in such manner that the circuit through the resistance 30 may be closed unless the water in the tank 17 is at least 20° C., or any other temperature that may be desired.

The thermostatic devices 36, 37, and 38 are adjusted to maintain the temperatures noted above in the tanks 18, 19 and 20, respectively, or any other temperatures that may be desired.

Briefly, in the operation of the above described apparatus, the tubing 11 passes from the extruding mechanism 10 through the tanks 15 and 16 into the first wash tank 17 and thence through the wash tanks 18, 19 and 20 into the tank 21 which holds the hygroscopic agent. The temperature of the water

in the tanks 17, 18, 19 and 20 is controlled by the thermostatic devices 35, 36, 37 and 38, respectively, in the manner described above so that the casing or tubing is not subjected to a high temperature immediately after it reaches the tank 16, but is gradually subjected to higher temperatures until it has been thoroughly washed.

While I have shown and described certain embodiments of my invention, it is to be understood that it is capable of many modifications. Changes, therefore, in the construction and arrangement may be made without departing from the spirit and scope of the invention as disclosed in the appended claims, in which it is my intention to claim all novelty inherent in my invention as broadly as possible, in view of the prior art.

I claim:

- 20 1. The method of forming a cellulose product, which method comprises extruding viscose and regenerating it and subjecting the regenerated viscose to several baths of heated water of increasing temperature.
- 25 2. The method of forming a cellulose product, which method comprises extruding viscose, regenerating it, and washing the regenerated substance in several baths of heated water of increasing temperatures, one of said baths being maintained at a temperature less than 40° C. and another of said baths being maintained at a temperature in excess of 40° C.
- 30 3. The method of forming a cellulose product, which method comprises extruding viscose, regenerating said viscose, and washing the regenerated substance in at least three baths of heated water of increasing temperatures, at least one of said baths being maintained at a temperature in excess of 35° C.

In testimony whereof, I hereunto affix my signature this 24th day of October, 1930.

WILLIAM F. HENDERSON.

45

50

55

60